

## UNITED STATES PATENT OFFICE.

LOUIS SPENCER FLATAU, OF ST. LOUIS, MISSOURI.

## PAINT COMPOUND.

SPECIFICATION forming part of Letters Patent No. 789,600, dated May 9, 1905.

Application filed December 19, 1904. Serial No. 237,576.

*To all whom it may concern:*

Be it known that I, LOUIS SPENCER FLATAU, a citizen of the United States, residing at St. Louis, State of Missouri, have invented new 5 and useful Improvements in Paint Compounds, of which the following is a specification.

My invention relates to an improved paint compound. It is designed more especially 10 for use upon and for treating heated metal surfaces, more particularly the front ends and stacks of locomotive and other engines and like purposes.

Said invention consists of the compound- 15 ing, substantially as and in the proportions hereinafter named, of certain ingredients presently described, and particularly pointed out by the claim.

In the carrying out of my invention I suit- 20 ably grind or reduce a quantity of crude gilsonite or asphaltum to the requisite fineness unattended with any heating action, thus preserving it intact and from loss of any of its properties, as would be the case in effecting 25 the reduction of the material by the use of fire or heat, which would be also more or less hazardous. The thus-ground gilsonite is run into a mixing-mill below, such as disclosed in my pending application filed De- 30 cember 19, 1904, Serial No. 237,575, into which latter has been previously placed about six barrels of naphtha. About eight barrels of the gilsonite are run into the mixing-mill, further quantities of the naphtha being added 35 as the quantity of gilsonite may require in order to regulate the gravity of the asphaltum composition or product. About ten barrels of the naphtha are finally put into the mixing-mill with the gilsonite to secure the de- 40 sired or effective product. Into this mixture I place two or three barrels of linseed-oil after having been boiled and then add two barrels of what is commonly called "gloss-oil," preferably prepared as later noted, and any good 45 drier. Said mixing-mill is suitably covered to prevent evaporation or escape of gases to annoy the attendants or workman and after

the whole has become thoroughly amalgamated into a perfect asphaltum composition, as it were, which is effected by rapidly running or rotating the mill. In the production of said gloss-oil I suitably reduce or comminute, as finely as may be required, crude rosin and run it into a mill—such, for instance, as herein designated—which has been suitably 50 supplied with benzin and dissolve the rosin therein by agitation unaided by any heating action, and as the oil is thus produced run it into barrels for use as needed.

My aforesaid paint compound, which is 60 characterized in its application by a black glossy surface, will effectively resist six or seven hundred degrees of heat, and is therefore, as I have found by actual use, highly 65 serviceable for painting, especially the front 70 ends of smoke-stacks of locomotive and other engines, as well as for all steel or wood work and which is incomparable for durability and appearance, while, as previously noted, the element of the use of fire in its manufacture 75 is entirely eliminated, which would be greatly objectionable for the reasons as aforesaid herein given.

Latitude is allowed as to details herein, as the same may be varied as circumstances 75 suggest without departing from the spirit of my invention.

I claim—

The herein-described process of producing a paint compound, which consists in reduc- 80 ing gilsonite by grinding to a powder; combining with naphtha said gilsonite in powder form by sifting the latter upon said naphtha; and adding to the aforesaid ingredients boiled linseed-oil and gloss-oil, and then thoroughly amalgamating this mixture 85 by the agitating action of a mill.

In testimony whereof I affix my signature in presence of two subscribing witnesses.

LOUIS SPENCER FLATAU.

Witnesses:

J. V. MUSICK,  
Wm. H. Scott.